

April 29, 1924.

1,492,255

B. McCAFFREY

METHOD OF RESURFACING OLD CONCRETE ROADWAYS

Filed July 25, 1923

*Sweep and clean, and wash roadway surface  
with naphtha or any other grease or oil remover.*



Fig. 1

*Checker or mark roadway surface  
and apply asphaltic paint coat*



Fig. 2

Fig. 3.



*Lay wearing surface  $\frac{3}{4}$ " to  $1\frac{1}{2}$ " thick*



Fig. 4.

Inventor

Berlin McCaffrey

*B. D. McCaffrey*

Attorney

## UNITED STATES PATENT OFFICE.

BERTIN McCAFFREY, OF WEST HOBOKEN, NEW JERSEY.

## METHOD OF RESURFACING OLD CONCRETE ROADWAYS.

Application filed July 25, 1923. Serial No. 653,806.

*To all whom it may concern:*

Be it known that I, BERTIN McCAFFREY, a citizen of the United States, residing at West Hoboken, in the county of Hudson and State of New Jersey, have invented certain new and useful Improvements in Methods of Resurfacing Old Concrete Roadways, of which the following is a specification.

10 My invention is a method of resurfacing old concrete roadways.

An important object of the invention is to provide a method of the above mentioned character, whereby old concrete roadways, 15 when worn, may be restored by providing the same with an asphalt surface coat, of a proper thickness, such coat being securely anchored or bonded to the old concrete roadway, in a manner to prevent separation, 20 creeping or slipping.

A further object of the invention is to provide a method of the above mentioned character, adapted for applying the asphalt surface coat to a concrete roadway having 25 no curb.

Other objects and advantages of the invention will be apparent during the course of the following description.

In the accompanying drawings, forming a 30 part of this specification, and in which like numerals are employed to designate like parts throughout the same,

Figure 1 is a vertical transverse section through a concrete roadway, illustrating the 35 cleaning of the roadway,

Figure 2 is a similar view illustrating the checkering or marking of the concrete roadway and the applying of the asphaltic paint.

Figure 3 is a plan view of the same, and, 40 Figure 4 is a transverse vertical section through the completed roadway, showing the application of the asphalt surface coat.

In accordance with my method, the old concrete roadway 5 has its surface mechanically cleaned, as by sweeping, for removing therefrom substantially all of the solid foreign matter, such as dirt, dust, etc. It is preferred that the sweeping be done thoroughly, so that substantially all of the 45 solid foreign matter may be removed, or as much removed as is practicable.

After the sweeping or cleaning of the solid foreign matter has been completed, the next step in the method is to wash the surface of the concrete roadway, with a liquid which will remove oils and greases. I preferably employ for this purpose naphtha, or any other grease or oil remover. This washing may be effected by means of brooms, mops, or by any manual or mechanical means, desired. The washing is preferably done in a thorough manner for removing substantially all traces of the oil or grease from the concrete roadway, or as much thereof as is practicable.

The old concrete roadway thus thoroughly cleaned of all oils or greases, next has its surface roughened. This is preferably accomplished by checkering, marking or grooving the surface, as indicated at 6, 10 by using a scarifier, or by means of any other hand method or mechanical device, which may be practicable. The checkering or marking consists in forming indentations in the face of the concrete roadway, which 15 indentations may extend over substantially the entire surface of the roadway, or a part thereof. The checkering or marking of the roadway is preferably distributed uniformly through the entire area of the same, but 20 the fineness of the checkering or marking may vary somewhat, as may be found advantageous. It is ordinarily preferred that the checkering or marking be sufficient to roughen up the greater portion or substantially all of the roadway, thereby leaving the 25 same clean, with fresh indentations in the whole or part of the same.

I also form channels 7 in the surface of the concrete roadway, except where curbs are used. The function of these channels is to securely bond the surface coat, to be described, to the roadway.

After the roadway is thus checkered, marked, or roughened, the next step in the method consists in applying thereto an asphaltic paint coat, which is applied to the entire surface thereof, by means of a brush or any other suitable means. This asphaltic paint coat, at atmospheric temperature, is 50 of a heavy plastic consistency, and in order to apply the same to the concrete roadway,

it must be first heated so that it is rendered fluid. In this heated fluid condition it may be splashed upon the roadway, or applied by means of a brush. The asphaltic paint 5 may also be rendered fluid, without heating, by dissolving the same in a suitable amount of naphtha, which would then produce a fluid known in the trade as a cut back asphalt. This liquid may be applied with a brush or 10 by splashing, or by any other suitable means. This asphaltic paint mixes with the asphalt in the asphalt surface coat, to be described, and leads the same into the crevices or pores 15 of the concrete. The function of this asphaltic paint coat is to aid in the adhesion of the asphalt surface coat, which is subsequently applied, so that the shoving or creeping 20 of the asphalt surface coat is prevented.

After the concrete roadway is thus treated, 25 and with the asphalt paint applied thereto, the next step in the method is the laying thereon of an asphalt surface coat 8, which preferably has the thickness of from  $\frac{3}{4}$  of an inch to  $1\frac{1}{2}$  inches.

25 The asphalt used in the asphalt surface coat shall be of any standard type or brand manufactured for paving purposes, and shall preferably have a penetration of from 40 to 60 under No. 2 needle at  $77^{\circ}$  F.-5 seconds, 30 100 grams, and it is preferred that the penetration shall not vary outside of these limits, except when climatic conditions make it necessary to vary the same above these limits.

35 The asphalt surface coat embodies mineral aggregates, and asphaltic or bituminous material. The mineral aggregate should preferably consist of broken stone, gravel, sand, or other suitable material, so that the same may meet one of the following mesh compositions, in the finished coat or surface mixture:

*Coat surface mixture "A".*

| 45 | Mineral aggregate.       | Percentage of total mixture as laid. |  |
|----|--------------------------|--------------------------------------|--|
|    |                          | Per cent.                            |  |
|    | Passing 200 mesh screens | 5 to 11                              |  |
|    | " 40 "                   | 18 to 30                             |  |
|    | " 10 "                   | 25 to 55                             |  |
|    | " 4 "                    | 8 to 22                              |  |
| 50 | " 2 "                    | Not less than 10                     |  |
|    | Asphaltic cement         | 7 to 11                              |  |

*Coat surface mixture "B".*

| 55 | Bitumen                  | 7 to 11 per cent.                    |
|----|--------------------------|--------------------------------------|
| 60 | Mineral aggregate.       | Percentage of total mixture as laid. |
|    | Passing 200 mesh screens | Per cent.                            |
|    | " 80 "                   | 5 to 12                              |
|    | " 40 "                   | 10 to 20                             |
|    | " 10 "                   | 8 to 25                              |
|    | " 4 "                    | 25 to 50                             |
|    | " 2 "                    | 8 to 22                              |
|    |                          | 0 to 10                              |

*Coat surface mixture "C".*

65 Bitumen..... 9.5 to 13.5 per cent.

| Mineral aggregate.                | Percentage of total mixture as laid. | 70 |
|-----------------------------------|--------------------------------------|----|
| Passing 200 mesh                  | Per cent.                            |    |
| " 80 "                            | Not less than 10                     |    |
| " 50 "                            | 10 to 35                             |    |
| " 40 "                            | 4 to 35                              |    |
| " 30 "                            | 4 to 25                              |    |
| " 20 "                            | 4 to 20                              |    |
| " 10 "                            | 2 to 12                              | 75 |
| " 8 "                             | 0 to 5                               |    |
| Total passing 200, 11 and 80 mesh | Not less than 25                     |    |
| " " 50, and 40 "                  | 15 to 50                             |    |
| " " 30, 20 and 10 "               | 10 to 35                             |    |

*Coat surface mixture "D".*

| Mineral aggregate.                               | Percentage of total mixture as laid. | 80 |
|--------------------------------------------------|--------------------------------------|----|
| Retained by 10 mesh sieve                        | Per cent.                            |    |
| Passing 10 mesh sieve, retained by 40 mesh sieve | None                                 | 85 |
| " 40 "                                           | 10 to 35                             |    |
| " 80 "                                           | 20 to 65                             |    |
| " 200 "                                          | 15 to 30                             |    |
| Bitumen                                          | 12 to 20                             |    |
|                                                  | 9 to 12.5                            |    |

90 The asphalt surface coat also embodies a mineral filler, which is Portland cement, or limestone dust filler. This mineral filler is added to the mix in a suitable per cent to bring the finest of the mineral aggregate, 95 stated for the purpose of illustration as passing 200 mesh screens, up to between the limits of the per cent stated, as may be desired. For instance, in the surface coat mix "A" if only 2 per cent of the mineral aggregate passes through the 200 mesh screens, then not less than 3 per cent or more than 9 per cent of the mineral filler will be added.

95 The mineral aggregate shall be heated in the following manner, and the asphalt shall 105 also be heated in a manner to be described. The mineral aggregate for the surface coat shall be heated, before entering the mixer, to between  $225^{\circ}$  and  $350^{\circ}$  F., in a revolving drier of any approved type, in which no flame 110 shall be permitted to come in contact with the aggregate. The aggregate shall be continuously agitated during the heating. This heated mineral aggregate is then conveyed to a suitable hopper which may be located 115 above a rotatable mixer. The desired amount of the mineral aggregate may be withdrawn into the rotatable mixer, and then the fine mineral filler, passing the 200 mesh screens, is introduced cold into the 120 mixer with the mineral aggregate, in the suitable per cent. The asphalt or asphalt cement furnished for the surface coat shall be heated separately from the mineral aggregate in approved receptacles so designed 125 as to admit of an even heating of the entire mass, with an efficient and positive control of the heat at all times. This asphalt cement

shall be heated to the temperature directed from time to time between 250° and 350° F. This heated asphalt cement, which is now in a liquid condition, is now introduced into the mixer with the mineral aggregate and mineral filler, and the entire mass is thoroughly agitated, until the same becomes homogeneous. The mixing shall continue until every particle of the mineral aggregate and mineral filler is completely coated with the asphalt cement, and a uniform mixture has been obtained. The mass when discharged from the mixer retains a temperature of from not more than 350° F. and not less than 225° F.

The asphalt surface coat, heated and prepared as above described shall be delivered from the mixer to the point of deposition in the pavement, in suitable trucks or wagons, provided with canvas covers for retaining the heat. As delivered to the point of application to the roadway, the asphalt surface coat shall have a temperature of at least 225° F. The material having a lower temperature than 225° F. shall not be laid in the surface coat. The asphalt surface coat mixture shall be immediately spread over the concrete roadway, by men experienced in such work, so that when rolled it shall have a thickness at no place less than  $\frac{3}{4}$  of an inch, or more than  $1\frac{1}{2}$  inches, and shall be free from surface depressions and irregularities.

The asphalt surface coat, when placed as above described, shall be rolled at once, while the material is still warm and pliable, the rolling beginning at the edges in the roadway and working toward the center. Suitable means shall be provided to prevent the asphalt surface coat sticking to the roller. Rolling shall continue without interruption until all roller marks disappear and the surface shows a uniform compressibility. Places which the roller cannot effectively reach shall be compressed with heated iron tamps.

Rollers used for compressing the asphalt surface coat shall be well-balanced, self-propelled tandem or three-wheel rollers of satisfactory design, weighing preferably between ten and fifteen tons each.

The asphalt surface coat is applied to the concrete roadways, immediately after the application of the asphaltic paint coat. This paint coat serves to lead the asphalt surface coat into the crevices, pores or the like of the concrete. This action is also aided by the pressure of the rollers. The result of the combined action of the several steps of the method, is the maximum binding action between the asphalt surface coat, and concrete roadway.

While it is believed that more satisfactory results are obtainable by employing all of the methods of the invention, in the treat-

ing of the roadway, yet it has been found that in some instances, the roughening of the cleaned roadway may be dispensed with, and some degree of success obtained. Also, it has been found that the coating of the roughened roadway with the asphaltic paint may be dispensed with, in some instances, with some degree of success.

While the drawing shows the surface of the concrete roadway checkered diagonally, it is obvious that the invention is in no sense restricted to this method of checker- 75 ing, as the roadway may be roughened in any manner desired. The checkerling may be arranged longitudinally, transversely, or in an irregular manner, if desired.

It is to be understood that the form of my invention herewith shown and described, is to be taken as a preferred example of the same, and that various changes in the order of the steps of the method, and that equivalent steps may be employed, without departing from the spirit of my invention, or the scope of the subjoined claims.

Having thus described my invention, I claim:

1. The method of effecting a close bond or union between the surface of an old or worn concrete roadway and an asphalt surface coat mixture to be applied thereto, so that the asphalt surface coat mixture thus applied will not slip or creep, by sweeping the surface of the old or worn concrete roadway for removing foreign solid material, washing such surface with a solvent of oil and grease to remove the same, roughening the cleaned surface thus treated, applying to the roughened cleaned surface an asphalt paint coat, applying to the surface thus coated a heated asphalt surface coat mixture embodying mineral ag- 95 gregates coated with asphalt, and then rolling the asphalt coat surface mixture while it is compressible.

2. The method of effecting a close bond or union between the surface of an old or worn concrete roadway and an asphalt surface coat mixture to be applied thereto, so that the asphalt surface coat mixture thus applied will not slip or creep, by sweeping the surface of the old or worn concrete roadway for removing foreign solid material, cutting such surface for producing anchor indentations, applying to the surface thus treated a liquid adapted to serve as a binder for an asphalt surface coat 110 mixture, applying to the coated surface a heated asphalt surface coat mixture, and rolling the asphalt surface coat mixture 120 while it is compressible.

3. The method of effecting a close bond or union between the surface of an old or worn concrete roadway and an asphalt surface coat mixture to be applied thereto,

so that the asphalt surface coat mixture thus applied will not slip or creep, by sweeping and washing the surface of the old or worn concrete roadway for the removal of solid matter and grease, roughening the cleaned surface, applying to the roughened surface an asphalt paint coat binder, applying to the surface thus coated a heated asphalt surface coat mixture, and then rolling the asphalt coat surface mixture while it is compressible.

4. The method of effecting a close bond or union between the surface of an old or worn concrete roadway and an asphalt surface coat mixture to be applied thereto, so that the asphalt surface coat mixture thus applied will not slip or creep, by cleaning the surface of the old or worn concrete roadway to remove foreign matter, roughening the cleaned surface, forming longitudinal channels near the outer edges of the roadway, applying to the surface of the roadway thus treated a heated asphalt surface coat mixture, and then rolling the asphalt surface coat mixture while compressible whereby it becomes securely anchored within the roughened portions of the surface and the channels.

5. The method of effecting a close bond or union between the surface of an old or worn concrete roadway and an asphalt surface coat mixture to be applied thereto,

so that the asphalt surface coat mixture thus applied will not slip or creep, by sweeping and washing the surface of the old or worn concrete roadway for removing solid matter and grease or oil, cutting anchor indentations in such surface, forming longitudinal channels near the longitudinal outer edges of the roadway, applying to the surface thus treated a heated asphalt surface coat mixture, and then rolling the asphalt surface coat mixture.

6. The method of effecting a close bond or union between the surface of an old or worn concrete roadway and an asphalt surface coat to be applied thereto, so that the asphalt surface coat thus applied will not slip or creep, by cleaning the surface of the concrete roadway, removing solid and greasy matter, roughening the cleaned surface of the concrete roadway, applying to the roughened surface of liquid which serves to lead the asphalt surface coat into the pores of the concrete roadway and into the crevices of the roughened surface, applying an asphalt surface coat mixture to the coated surface and working the asphalt surface coat mixture well into the roughened surface of the concrete roadway.

In testimony whereof I affix my signature.

BERTIN McCAFFREY.